

Dec. 17, 1929.

M. LEVIN

1,740,184

CLOSURE FOR RECEPTACLES

Filed April 27, 1927

*Fig. 1.*



*Fig. 2.*



*INVENTOR*  
*M. Levin*  
*BY*  
*Sigmund Hergott*  
*ATTORNEY*

## UNITED STATES PATENT OFFICE

MICHAEL LEVIN, OF BROOKLYN, NEW YORK

## CLOSURE FOR RECEPTACLES

Application filed April 27, 1927. Serial No. 186,969.

The present invention relates to improvements in closures for receptacles, and more particularly to closures of the cap variety. Closures of this type comprise usually a metallic cap and a sealing disk or packing of cork, pasteboard or the like, the shell and packing being stuck together by an interposed cementing medium.

In manufacturing crown corks, which are closures of the cap variety, two types of cementing materials have been used heretofore. One of these types is fusible by heat and the other type is coagulable by heat. When fusible material is employed, it is placed into the cap, the packing disk being put on top of the cementing material and the assembled closure subjected to heating action to fuse the cementing material, the elements of the closure being maintained under pressure while the cementing material is caused to set or harden, whereby the sealing disk is united with the metallic cap. When a coagulable cementing material is employed, the assembled closure is heated under pressure, whereby the cementing material coagulates and unites the elements of the closure.

Coagulable cementing materials are albuminous substances, egg albumen or blood albumen, or a combination of both, or casein having been employed heretofore in the art of making closures.

The present invention relates to closures in which albuminous substances are employed as cementing media.

The egg albumen or blood albumen, both as found on the market as a granular product, have been heretofore dissolved in water, each closure cap being charged with a measured quantity of the product so obtained, a sealing disk or packing being then inserted into the cap on top of the cementing medium, and the assembled closure placed under pressure and heated. The heat coagulates the cementing medium and renders it insoluble. The closures cannot be subjected to heat above 200° F., as any higher heat injures the packing and also affects the decorations or printing on the outer surfaces of the caps. The machines on which these closures are assembled and united must be run, therefore, consider-

ably slower than the assembling and uniting operations require, the speed being determined by the time required to coagulate the cementing material. Both egg albumen and blood albumen have also been found objectionable on the ground that they have a tendency to decay or putrefy, and for this reason cementing materials containing blood albumen or egg albumen must be prepared from day to day and made use of immediately. Blood albumen is furthermore objectionable in preparing a cementing material for the purpose stated, because of its dark color.

The main object of the present invention is to provide a closure for receptacles in which the cementing material consists of a heat-coagulable substance in the form of rubber latex, with which may be mixed egg albumen or blood albumen, or a combination of both, or casein, or other materials which are generally used as glue or cements.

One of the many possible embodiments of the invention is illustrated in the accompanying drawings, in which:—

Figure 1 is a central vertical section of a closure constructed in accordance with the present invention; and Fig. 2 is a similar section of a modified construction.

In the drawings a closure of the crown cork type has been shown for purposes of illustration. It is, however, obvious that the invention may be applied to all closures of the cap variety, the forms of the metallic caps thereof being entirely immaterial as far as the invention is concerned.

Referring now first to Fig. 1 of the drawings, the numeral 10 indicates a cap, comprising a substantially cylindrical head 11 and a corrugated flange 12, the latter being adapted to be locked, in the well known manner, to the exterior of a bottle neck. This cap is made as usual of thin sheet iron coated with tin, the outer face of its head being sometimes decorated. Within the cap is disposed a sealing disk or packing 13 of cork or the like, which is united with the cap by an interposed cementing medium, denoted by the numeral 14. The cementing material is coagulated and set, and also rendered insoluble, by heat

Latex may be used as the cementing material, either alone or it may be mixed with other substances, such as for instance egg albumen or blood albumen, or it may be mixed with casein or other materials which are generally used as glues or cements.

If latex and albumen are used as a cementing material, the albumen, such as egg albumen or blood albumen, is dissolved in water. To the solution is added rubber or like latex, with which has been mixed a preservative agent, such as ammonia, formaldehyde, etc. By the use of the term "latex" is meant any of the milky or laticiferous saps or juices obtained from trees and plants and as are contained in rubber, gutta-percha and balata, as well as including the various combined salts, minerals and other natural substances usually found therein. Latex is understood to be an emulsion or colloidal suspension of the several solid constituents in water. While all of these latices are adapted to be used in preparing the cementing material, it is preferred to use rubber-containing latex obtained from the *Hevea brasiliensis*, this being the tree from which most of the rubber gathered on the Amazon and its tributaries is obtained, and is also the tree which is most exclusively cultivated in Ceylon, Federated Malay States, Straits Settlements, Sumatra and other parts of the East. As above mentioned, either egg albumen or blood albumen may be used, both as found on the market as a granular product. It is preferred to use blood albumen, because it is considerably cheaper than egg albumen.

Preferably, the ingredients of the cementing material are combined in the proportions stated, viz: 8 lbs. of albumen are dissolved or swelled in 15 lbs. of water, and to the resultant material are added 2 lbs. of latex, the compound being thoroughly stirred and agitated to produce a homogenous product. It is obvious that, while herein specific proportions of the ingredients of the cementing material are mentioned, changes may be made according to the requirements.

In manufacturing the closure, the metallic cap is charged with the cementing material, a suitable quantity being deposited into the cap by some mechanical means, and afterwards the material deposited is spread over the entire inner surface of the head of the cap. The sealing disk or packing of cork or the like is then inserted into the cap on top of the cementing medium, the assembled closure subjected to pressure and exposed to heat. The heat causes the albumen to coagulate and the latex to set, thereby uniting the metallic cap with the sealing disk or packing. Both the albumen and the latex are rendered insoluble by the application of heat.

By adding latex to albumen, the coagulation of the latter is materially accelerated.

Actual experiments have shown that a period

of two seconds at a temperature of 200° F. produces the necessary coagulating effect on the albumen, when latex is present. In all closure making processes heretofore in use at least eleven seconds are required for coagulating the albumen. It will thus be observed that, by using the cementing material herein described, rapidity of binding may be effected in a manner not heretofore obtainable.

As stated above, blood albumen may be used in preparing the cementing material without any objectionable or detrimental effect on the food products in the containers to which the closures are applied. It has been found that the cheapest grade of blood albumen may be used and yet the cementing material will be free from the ordinary objectionable dark color of the product, the ammoniated latex having a bleaching effect on the blood albumen.

Actual experiments have also shown that the ammonia in the latex acts on the albumen by causing it to go easily into the solution. The albumen, on the other hand, has an emulsifying action on the latex, preventing it from drying up. The cementing material may be prepared and left to stand for several days without putrefying or decomposing action setting in.

If necessary, a paper or other disk may be interposed between the metallic cap and the sealing disk. A structure of this type is shown in Fig. 2 of the drawings, comprising a cap 15, having disposed therein a disk 16 of paper or similar material, which is stuck to the cap by the cementing material above described and denoted by the numeral 17. Upon this disk may be placed a sealing disk 18 of cork or the like, joined with the disk 16 by cementing material 19 of the character above specified. In such cases the cap is first charged with a suitable quantity of cementing medium, the paper disk placed on top of it, the exposed face of said paper disk coated with the cementing medium, after which the sealing disk is deposited into the cap and the assembled closure subjected to the treatment above described. If more convenient, the paper or other disk may be coated, before insertion, with the cementing medium.

The closures herein described are capable of being produced at a considerably lower cost than those heretofore made for two reasons, to wit: First, because they can be manufactured at a speed of operation heretofore unattainable and, second, because the cementing material is of exceedingly low cost, as it permits the use of the cheapest kind of blood albumen.

Instead of latex, water dispersions of rubber may be used, either alone or with the other ingredients mentioned herein, as a cementing material.

It is intended to include in the appended claims in the term "cementing medium" the said medium alone or a disk of paper or other material coated therewith. Furthermore by "latex" as used in the claims is meant the juices of plants producing rubber, gutta-percha or balata.

What I claim is:—

1. A closure for receptacles, comprising a metallic cap, a sealing disk, and an interposed cementing medium composed of a heat-coagulated material and a substance set by heat and which has a tendency to directly accelerate the coagulation of said first-mentioned material.

2. A closure for receptacles, comprising a metallic cap, a sealing disk, and an interposed cementing medium composed of a heat-coagulated albuminous material and a substance set by heat and which has a tendency to directly accelerate the coagulation of said albuminous material.

3. A closure for receptacles, comprising a metallic cap, a sealing disk, and an interposed cementing medium composed of a heat-coagulated material and latex set by heat.

4. A closure for receptacles, comprising a metallic cap, a sealing disk, and an interposed cementing medium composed of a heat-coagulated material and ammoniated latex set by heat.

5. A closure for receptacles, comprising a metallic cap, a sealing disk, and an interposed cementing medium composed of a heat-coagulated albuminous material and latex set by heat.

6. A closure for receptacles, comprising a metallic cap, a sealing disk, and an interposed cementing medium composed of a heat-coagulated albuminous material and ammoniated latex set by heat.

7. A closure for receptacles, comprising a metallic cap, a sealing disk, and an interposed cementing medium composed of a heat-coagulated material and preserved latex set by heat.

8. A closure for receptacles, comprising a metallic cap, a sealing disk, and an interposed cementing medium composed of a heat-coagulated albuminous material and preserved latex set by heat.

9. A closure for receptacles, comprising a metallic cap, a sealing disk, and an interposed cementing medium containing latex set by heat.

10. A closure for receptacles, comprising a metallic cap, a sealing disk, and an interposed cementing medium containing preserved latex set by heat.

11. A closure for receptacles, comprising a metallic cap, a sealing disk, and an interposed cementing medium containing ammoniated latex set by heat.

12. A closure for receptacles, comprising a metallic cap, a sealing disk, and an inter-

posed cementing medium composed of latex set by heat.

13. A closure for receptacles, comprising a metallic cap, a sealing disk, and an interposed cementing medium composed of preserved latex set by heat.

14. A closure for receptacles, comprising a metallic cap, a sealing disk, and an interposed cementing medium composed of ammoniated latex set by heat.

15. A process for the manufacture of closures which includes a cap and a sealing disk, the steps which comprise interposing a cold adhesive albuminous material containing latex between the cap and sealing disk, subjecting the two to pressure and directly heating the same at a temperature sufficient to coagulate the albuminous material.

16. A process for the manufacture of closures which includes a cap and a sealing disk, the steps which comprise interposing a cold adhesive albuminous material including an accelerator between the disk and cap, adhesively associating the parts by pressure and then heating the same to a temperature sufficient to coagulate the albuminous material.

17. A process for adhering non-metallic material to metallic material, such as making a closure for receptacles, the metallic material comprising a metallic cap and the non-metallic material comprising a sealing disk, the steps which comprise interposing a cold adhesive albuminous material containing latex between the metallic material and the non-metallic material, subjecting the two to pressure and directly heating the same at a temperature sufficient to coagulate the albuminous material.

18. A process for adhering non-metallic material to metallic material, such as making a closure for receptacles, the metallic material comprising a metallic cap and the non-metallic material comprising a sealing disk, the steps which comprise interposing a cold albuminous material including an accelerator between the metallic material and the non-metallic material, adhesively associating the parts by pressure, and then heating the same to a temperature sufficient to coagulate the albuminous material.

Signed at New York, in the county of New York and State of New York, this 27th day of January, A. D. 1927.

MICHAEL LEVIN. 120

125

130